

## 1

3,412,024

INHIBITION OF CORROSION OF METALS  
James R. Stanford, Houston, Tex., assignor to Nalco  
Chemical Company, Chicago, Ill., a corporation of  
Delaware  
No Drawing. Filed Apr. 7, 1964, Ser. No. 358,119  
7 Claims. (Cl. 252—8.55)

This invention, in general, relates to new chemicals; new corrosion inhibiting compositions useful in preventing or minimizing corrosion of iron or steel tubing, other well parts, and the like which come in contact with corrosive sweet and sour crude oils, especially those containing corrosive brines recovered with the oil; and to methods of inhibiting such corrosion.

An object of the invention is to provide new compounds useful, for example, in inhibiting corrosion of metal equipment in oil and gas wells.

Another object of the invention is to provide chemicals for use in preventing corrosion of pipe or equipment which is in contact with a corrosive oil-containing medium in oil wells, refineries or the like.

Still a further object of the invention is to provide corrosion-inhibiting chemicals for protecting metals in systems which are subject to contact by various corrosive agents such as carbon dioxide, aqueous or nonaqueous solutions of carbon dioxide, hydrogen sulfide, aqueous or nonaqueous solutions of hydrogen sulfide, brines, weak inorganic acids and organic acids.

A still further object is to provide methods of inhibiting corrosion of ferrous metals in contact with said corrosive media with the aforesaid chemicals.

An additional object of the invention is to provide new and improved corrosion inhibiting compositions which are readily adsorbed by metal surfaces. Other objects will appear hereinafter.

The new chemicals of the invention comprise alkylbenzene sulfonic acid salts of partial amides of organic polyamines and acyclic monocarboxylic acids and polycarboxylic acids containing 1—48 carbons and an acyclic chain which is either saturated or olefinically unsaturated. The acids further may comprise in part cyclic carboxylic acids, notably rosin acids, such as rosin acids existing in crude tall oil, the chief rosin acid of which is abietic acid. The partial amide is one in which at least one but less than all of the amino groups of the polyamine are amidified with the carboxylic acid or acids. At least one and up to all of the basic, nonamidified amino groups of the partial amide form amine salt groups with the alkylbenzene sulfonic acid when the sulfonic acid is mixed with the partial amide. The alkyl group of the alkylbenzene sulfonic acid should have 8—16 carbons, dodecylbenzene sulfonic acid being the preferred species.

The polyamines may be polyalkylene polyamines having 3 to about 10 amino groups and 2—6 carbon alkylene groups. There are a number of mixtures of these polyamines commercially available at reasonable costs. The polyamine may also be an aminoalkyl derivative of a basic N-heterocycle such as N-aminoalkyl piperazines wherein the alkyl group has 2—6 carbons and aminoalkyl homologs thereof wherein the N-substituent has the formula,  $H(HN—R—)_x$  wherein R is the alkylene group of 2—6 carbons and x is a small whole number greater than one. The sulfonic acid salts form on a basic nitrogen of said compounds.

## 2

In addition to the foregoing salts, the invention also embraces corrosion inhibiting compositions comprising mixtures of said partial amide salts and 10—150%, based on the weight of said salts, of free acyclic acids as afore-defined in pure form, in admixture with each other, or in admixture with rosin acids, e.g., crude tall oil.

Embodiments of the invention are illustrated in the following examples, wherein the parts or percentages stated are by weight unless otherwise stated. For sake of brevity, certain compounds or compositions in the examples are identified by trade name. These compounds are:

(1) Century D-1475 acid is a mixture of vegetable oil fatty acids (essentially  $C_{14}$ — $C_{18}$  fatty acids) having an acid value of 188—203, a saponification value of 190—210 and an iodine value of 40—50.

(2) Century D-75 acid is a mixture of polymerized vegetable fatty acids containing a major proportion of dimerized and trimerized linoleic and linolenic acids and having an acid value of 155—169, a saponification value of 186—192, and an iodine value of 40—48. Century D-85 acid is a similar mixture of polymerized vegetable fatty acids containing a high percentage of trimer. It has a saponification value of a range from 125—148 and an iodine range of 42—50.

(3) Emery 3363D acid is a mixture of polybasic acids derived from natural fats and oils. The acid mixture has an average of about two carboxyl groups per molecule, an acid value of 208, a saponification value of 252, and an iodine value of 11.

(4) Emery 3362D acid is a blend of low molecular weight acids of the fatty acid series from formic acid through heptanoic acid with formic acid in preponderance. The blend has an acid value of 690.

(5) TX-3650 is a mixture of organic acids obtained as a wax oxidate and having a saponification number of 440—450 and a neutralization number of 225—250.

(6) Amine AL-1 is a mixture of N-aminoethyl-piperazine, N-hydroxyethylpiperazine, N-aminoethylethanamine and higher homologs of these compounds. The mixture has a total nitrogen content of 29.7—30.8%, and a titratable amine content of 16.4 meg./gm.

(7) Emfac 1202 is a pelargonic acid which is the normal  $C_9$  fatty acid, having an acid value of 345—360 and an iodine value of 1 maximum.

## EXAMPLE I

In a three-necked reaction vessel equipped with a stirrer, a Dean-Stark trap, a condenser and a thermometer, there were added, in parts by weight, 150 parts of crude tall oil, 75 parts of a mixture of polyethylene polyamines containing polyethylene polyamines of the series  $H_2N—(RNH)_xH$  wherein the polyethylene polyamines are higher homologs than tetraethylene pentamine (Polyamine H Solid, Union Carbide and Carbon), and 50 parts of  $SO_2$  extract, an aromatic hydrocarbon solvent. The mixture was heated to 150° C. Aqueous distillate was removed from the heated reaction mixture in a period of fifteen minutes in an amount of about 10.5 parts, the temperature rising to about 250° C. The resultant amide reaction product in the solvent was cooled to 150° C., and another 200 parts of  $SO_2$  extract were added.

After the product cooled to about 80° C., it was stirred and blended with the following chemicals in the order stated:

- (1) 290 parts of dodecylbenzene sulfonic acid.
- (2) 580 parts of Emery 3363-D Acid.
- (3) 810 parts of  $\text{SO}_2$  extract.
- (4) 58 parts of methanol.
- (5) 35 parts of polyoxyethylated phenol formaldehyde resin (nonylphenol-formaldehyde resin consisting of approximately 43% resin with the balance polyoxyethylene groups).
- (6) 23 parts of an emulsion breaker, containing a blend of an ethoxylated nonyl phenol resin with a mixed ester of an oxyalkylated tripentaerythritol monoester.

## EXAMPLE II

The procedure of Example I was repeated with 270 parts of Century D-1475 Acid, 100 parts of diethylene triamine and 50 parts of  $\text{SO}_2$  extract. The aqueous distillate began to distill over at about 160° C. Thirty-seven parts of aqueous distillate were removed in a 23 minute period, during which the temperature rose to about 250° C.

After adding 200 parts of  $\text{SO}_2$  extract, the following were blended therewith in the order stated:

- (1) 350 parts dodecylbenzene sulfonic acid.
- (2) 230 parts of Century D-85 Acid.
- (3) 1830 parts  $\text{SO}_2$  extract.
- (4) 230 parts isopropyl alcohol.
- (5) 7 parts emulsion breaker of Example I.

## EXAMPLE III

The procedure of Example I was repeated with 125 parts of crude tall oil, 25 parts of the aforescribed Emery 3363-D Acid, 50 parts of the aforescribed Polyamine H Solid, and 50 parts of  $\text{SO}_2$  extract. The aqueous distillate began to distill over at about 167° C. Ten and one-half parts of aqueous distillate were collected in a 10-minute period, during which the temperature rose to 250° C. After cooling and adding 200 parts of  $\text{SO}_2$  extract, the following were added in the order stated:

- (1) 91 parts of dodecylbenzene sulfonic acid.
- (2) 91 parts of Emery 3363-D Acid.
- (3) 238 parts of  $\text{SO}_2$  extract.
- (4) 45 parts of isopropyl alcohol.
- (5) 18 parts of polyoxyethylated phenolformaldehyde resin of Example I.
- (6) 4 parts of an emulsion breaker of Example I.

The corrosion protection values in the following tables were determined by semi-dynamic corrosivity tests, also known as corrosion inhibitor "wheel tests." The degree of protection to be expected from corrosion inhibitors in the produced fluids from oil and gas wells can be evaluated by these tests. They further indicate the minimum dosage at which inhibitors are capable of laying down and maintaining protective films under laboratory conditions simulating well conditions, especially those where inhibitor application is continuous or semicontinuous.

This test evaluates the corrosivity of produced fluids by determining weight loss of metal specimens exposed in sealed vessels containing the fluids. The sealed vessels are mounted on a wheel or mounting-board and maintained under constant rotation and temperature throughout the exposure period.

The effectiveness of inhibitors is rated by comparing weight losses of similar specimens in inhibited and uninhibited samples of fluid.

## Procedure

Test cells are filled with fresh fluids at the same oil/water ratio as exists in the field samples. (If a sizeable vapor space exists in the sample bottles as received, the fluids in the bottles are purged with inert gas to remove oxygen. The purged samples then are saturated with carbon dioxide, if they are from sweet gas condensate wells, or are saturated with hydrogen sulfide, if they are from sour wells.)

Inhibitors for evaluation are introduced into the test

- 5 cells at various dosages. "Control" test cells containing no chemical also are used, to establish a base corrosion rate from which relative "percent protection" provided by the chemicals can be computed. All tests normally are run in duplicate.

Weighed metal specimens are inserted and the test cells mounted on a rotating "wheel." The sealed test vessels are maintained under constant temperature and rotation rate throughout the exposure.

Following exposure, the specimens are removed, degreased in acetone or benzene and then scrubbed with soap and water. If corrosion products adhere to the surface, they are removed by dipping the coupons in inhibited technical-grade hydrochloric acid. After cleaning, the coupons are immersed in alcohol, then in acetone or benzene, dried and reweighed.

(wt. loss uninhibited-wt. loss with inhibitor)  
wt. loss uninhibited

$$\times 100 = \text{percent protection}$$

General test conditions are as follows:

- (1) Volume of test cells 200 ml. (about 0.4 pint).
- (2) Surface area of specimen per unit volume ----- 11.41 sq. ft./bbl. (1 cm.<sup>2</sup>/15 ml.) maximum.
- (3) Temperature range Room temp. to 200° F.
- (4) Type specimen Mild steel plate or carbon steel rod.
- (5) Surface of specimen Sandblasted (plate) or polished (rod).
- (6) Exposure period 24 hours.
- (7) Rotation rate 24 r.p.m.

35 Corrosion rates determined in this test typically are in excess of rates encountered in the field. This acceleration and magnification of corrosive attack shows up differences between chemicals and thus is an effective screening procedure.

40 Experience indicates that the following rough correlation exists between corrosivity ratings on this test and actual corrosivity of fluids in the field:

TABLE Ia

- 45 Weight loss in this test: Typical corrosiveness in field
 

|                         |          |
|-------------------------|----------|
| Less than 10 milligrams | Mild     |
| 10-20                   | Moderate |
| More than 20            | Severe   |

50 The following rough correlations also appear to exist between percent protection as furnished by inhibitors in this laboratory test, and the performance of the inhibitors in the field:

TABLE Ib

- 55 Protection by inhibitor in lab tests: Inhibitor performance in field
 

|               |           |
|---------------|-----------|
| 90% or more   | Excellent |
| 75% to 89%    | Good      |
| 50% to 74%    | Fair      |
| Less than 50% | Poor      |

60 The tests in the following examples were conducted at about 160° F. with mild steel plate for about 24 hours in a 50/50 volume mixture of sweet brine and kerosene saturated with  $\text{CO}_2$  unless otherwise indicated.

## EXAMPLE IV

70 In the equipment described in Example I, 150 parts of crude tall oil, 65 parts of Amine AL-1 and 50 grams of about 160° F. with mild steel plate for about 24 hours in utes. Nine parts of aqueous distillate were distilled off. The resultant ester-amide was diluted with 200 parts of toluene after it cooled. The resultant amide-ester solution, hereafter abbreviated A.E.S., was tested in the same 50/50  $\text{CO}_2$  saturated kerosene sweet brine corrosive mixture as a corrosion inhibitor in the following compositions.

TABLE II.—CORROSION RESULTS

| Composition in Parts By Weight                                           | Percent Protection at Concentration in p.p.m. |           |           |           |           |            |
|--------------------------------------------------------------------------|-----------------------------------------------|-----------|-----------|-----------|-----------|------------|
|                                                                          | 10 p.p.m.                                     | 20 p.p.m. | 40 p.p.m. | 60 p.p.m. | 80 p.p.m. | 100 p.p.m. |
| All A.E.S.                                                               | 11                                            | 7         | 21        | 18        | 18        | 29         |
| 40 A.E.S., 30 D.B.S.A., <sup>1</sup> 10 Century D-1475 Acid,             |                                               |           |           |           |           |            |
| 20 Toluene                                                               | 22                                            | 24        | 76        | 96        | 97        | 99         |
| 40 A.E.S., 30 D.B.S.A., <sup>1</sup> 10 Century D-85 Acid,               |                                               |           |           |           |           |            |
| 20 Toluene                                                               | 27                                            | 23        | 92        | 91        | 96        | 99         |
| 40 A.E.S., 30 D.B.S.A., <sup>1</sup> 25 Century D-1475 Acid,             |                                               |           |           |           |           |            |
| 30 Toluene                                                               | 28                                            | 36        | 92        | 99        | 98        | 99         |
| 40 A.E.S., 30 D.B.S.A., <sup>1</sup> 30 TX 3650, 30 Solvent <sup>2</sup> | 28                                            | 29        | 95        | 99        | 97        | 98         |
| 40 A.E.S., 40 Century D-1475 Acid, 20 Toluene                            | 0                                             | 21        | 35        | 62        | 98        | 99         |

<sup>1</sup> and <sup>2</sup>=Dodecylbenzene sulfonic acid and substitute SO<sub>2</sub> extract, respectively.

## EXAMPLE V

15

In the equipment described in Example I, 150 parts of crude tall oil, 65 parts of Amine AL-1 and 50 parts of substitute SO<sub>2</sub> extract were heated to 243° C. in a period of 73 minutes. Eleven parts of water were distilled off. The cooled amide-ester mixture was diluted with 200 parts toluene. The resultant ester-amide solution was blended at a ratio of 300 parts of said solution with 225 parts of dodecylbenzene sulfonic acid and 150 parts of substitute SO<sub>2</sub> extract. This product is hereafter designated "Blend."

Corrosion test results were:

TABLE III.—CORROSION RESULTS

| Composition in Parts By Weight  | Percent Protection at Concentration in p.p.m. |           |           |           |           |
|---------------------------------|-----------------------------------------------|-----------|-----------|-----------|-----------|
|                                 | 10 p.p.m.                                     | 20 p.p.m. | 30 p.p.m. | 40 p.p.m. | 50 p.p.m. |
| Blend (all)                     | 10                                            | 21        | 57        | 79        | 80        |
| 45 Blend, 5 Caprylic acid       | 41                                            | 25        | 38        | 79        | 85        |
| 45 Blend, 5 Capric acid         | 10                                            | 33        | 74        | 89        | 87        |
| 45 Blend, 5 Lauric acid         | 18                                            | 20        | 60        | 83        | 92        |
| 45 Blend, 5 Palmitic acid       | 15                                            | 33        | 78        | 90        | 90        |
| 45 Blend, 5 Century D-1475 Acid | 12                                            | 73        | 89        | 93        | 91        |
| 45 Blend, 5 Crude tall oil      | 14                                            | 22        | 74        | 87        | 88        |
| 45 Blend, 5 Century D-75 Acid   | 17                                            | 70        | 82        | 88        | 90        |
| 45 Blend, 5 TX 3650 Acid        | 11                                            | 37        | 91        | 92        | 93        |
| 45 Blend, 5 Acinto FA-1         | 12                                            | 19        | 72        | 89        | 90        |
| 40 Blend, 10 Caprylic Acid      | 16                                            | 14        | 70        | 75        | 75        |
| 40 Blend, 10 Palmitic acid      | 12                                            | 11        | 56        | 83        | 81        |

## EXAMPLE VI

In equipment described in Example I, a mixture of<sup>45</sup>

The resultant blend is designated in Table V as "Blend." The results of the corrosion tests were:

TABLE V.—CORROSION RESULTS

| Composition in Parts By Weight  | Percent Protection at Concentration in p.p.m. |           |           |           |           |
|---------------------------------|-----------------------------------------------|-----------|-----------|-----------|-----------|
|                                 | 10 p.p.m.                                     | 20 p.p.m. | 30 p.p.m. | 40 p.p.m. | 50 p.p.m. |
| Blend (all)                     | 0                                             | 18        | 26        | 39        | 35        |
| 45 Blend, 5 Lauric acid         | 10                                            | 16        | 33        | 27        | 35        |
| 45 Blend, 5 Century D-1475 Acid | 3                                             | 14        | 42        | 96        | 98        |

135 parts of Century D-1475 Acid (vegetable fatty acids), 50 parts of diethylene triamine and 50 parts of substitute SO<sub>2</sub> extract was heated to 240° C. in 18 minutes. Seventeen parts of water were distilled off. The cooled reaction mixture was diluted with 200 parts toluene.

Two hundred parts of the resultant solution were blended with 113 parts of dodecylbenzene sulfonic acid. The pH of the blend was about 6.0. The product is designated in Table IV as "Blend."

The corrosion test results were:

60

65

Using the equipment described in Example I, a mixture of 135 parts of Century D-1475 Acid, 66 parts of dipropylene-1,2-triamine and 50 parts of substitute SO<sub>2</sub> extract were heated to 242° C. in 20 minutes. Twenty-three parts of aqueous distillate were distilled over. Upon cooling, the partial amide was diluted with 200 parts of toluene. The amide solution was blended at a ratio of 100 parts of said solution with 40 parts of dodecyl-

TABLE IV

| Composition in Parts By Weight  | Percent Protection at Concentration in p.p.m. |           |           |           |           |
|---------------------------------|-----------------------------------------------|-----------|-----------|-----------|-----------|
|                                 | 10 p.p.m.                                     | 20 p.p.m. | 30 p.p.m. | 40 p.p.m. | 50 p.p.m. |
| Blend (all)                     | 2                                             | 23        | 40        | 82        | 79        |
| 45 Blend, 5 Lauric acid         | 5                                             | 30        | 56        | 92        | 95        |
| 45 Blend, 5 Century D-1475 Acid | 2                                             | 48        | 77        | 93        | 95        |

benzene sulfonic acid. The blend is designated in Table VI as "Blend."

The results of the corrosion tests were:

TABLE VI.—CORROSION RESULTS

| Composition in Parts By Weight       | Percent Protection at Concentration in p.p.m. |              |              |              |              |
|--------------------------------------|-----------------------------------------------|--------------|--------------|--------------|--------------|
|                                      | 10<br>p.p.m.                                  | 20<br>p.p.m. | 30<br>p.p.m. | 40<br>p.p.m. | 50<br>p.p.m. |
| Blend (all).....                     | 1                                             | 20           | 37           | 48           | 64           |
| 45 Blend, 5 Lauric acid.....         | 0                                             | 18           | 35           | 47           | 81           |
| 45 Blend, 5 Century D-1475 Acid..... | 0                                             | 21           | 39           | 88           | 93           |

## EXAMPLE IX

Using the equipment described in Example I, a mixture of 162 parts of Emfac 1202, 131 parts of dipropylene-1,2-triamine and 100 parts of substitute  $\text{SO}_2$  extract were heated to 240° C. in 30 minutes. Forty-six parts of aqueous distillate were distilled over. Upon cooling, the partial amide was diluted with 400 parts of toluene. The amide solution was blended at a ratio of 100 parts of said solution with 52 parts of dodecylbenzene sulfonic acid. The blend is designated in Table VII as "Blend."

The results of the corrosion tests were:

TABLE VII.—CORROSION RESULTS

| Composition in Parts By Weight       | Percent Protection at Concentration in p.p.m. |              |              |              |              |
|--------------------------------------|-----------------------------------------------|--------------|--------------|--------------|--------------|
|                                      | 10<br>p.p.m.                                  | 20<br>p.p.m. | 30<br>p.p.m. | 40<br>p.p.m. | 50<br>p.p.m. |
| Blend (all).....                     | 1                                             | 17           | 25           | 21           | 37           |
| 45 Blend, 5 Lauric acid.....         | 1                                             | 19           | 19           | 30           | 25           |
| 45 Blend, 5 Century D-1475 Acid..... | 3                                             | 11           | 25           | 44           | 91           |

## EXAMPLE X

In equipment described in Example I, a mixture of 150 parts of crude tall oil, 65 parts of Amine AL-1 and 50 parts of substitute  $\text{SO}_2$  extract was heated to 243° C. in 14 minutes. There were 10 parts of aqueous distillate. Upon cooling, the product was blended with 300 parts of substitute  $\text{SO}_2$  extract.

The product was blended at a ratio of 100 parts of the solution with 51 parts of dodecylbenzene sulfonic acid. The blend is designated in Table VIII as "Blend."

The corrosion results were:

TABLE VIII.—CORROSION RESULTS

| Composition in Parts By Weight       | Percent Protection at Concentration in p.p.m. |              |              |              |              |
|--------------------------------------|-----------------------------------------------|--------------|--------------|--------------|--------------|
|                                      | 10<br>p.p.m.                                  | 20<br>p.p.m. | 30<br>p.p.m. | 40<br>p.p.m. | 50<br>p.p.m. |
| Blend (all).....                     | 0                                             | 14           | 32           | 38           | 47           |
| 45 Blend, 5 Lauric acid.....         | 0                                             | 13           | 33           | 38           | 55           |
| 45 Blend, 5 Century D-1475 Acid..... | 0                                             | 15           | 34           | 81           | 87           |

The corrosion inhibiting chemicals and compositions herein disclosed are dispersed or dissolved in the produced fluids at concentrations ranging from 10 to 100,000 p.p.m. Corrosion inhibition may be achieved by either a continuous low concentration of inhibitor being in contact with the metal to be protected, or by using a high concentration of inhibitor in a batch or squeeze type treatment. When the chemical is applied continuously the concentration of inhibitor in the fluid falls within the preferred range of 10 to 500 p.p.m. When the chemical is used in a squeeze or batch type treatment the preferred range falls within 10,000 to 100,000 p.p.m. To those skilled in the art it will be apparent that the squeeze applications gives long term protection with single treatments.

The invention is hereby claimed as follows:

1. Corrosion inhibiting compositions wherein the active, corrosion inhibiting compounds consist essentially of (A) salts of (a) alkylbenzene sulfonic acids having 8-16 carbon alkyl groups and (b) partial amides of at least one of monomeric, dimeric and trimeric higher fatty acids and organic amines having a plurality of basic nitrogens, substantially all of which are in the form of amine salt groups with said alkylbenzene sulfonic acids, said amines selected from the group consisting of polyalkylene polyamines having 3-10 amino groups and 2-6 carbon alkylene groups and N-aminoalkyl substituted piperazines wherein the aminoalkyl group has the formula  $H(HNR—)_x$  wherein R is an alkylene group of 2-6 carbons and x is a small whole number, and (B) 10-150% by weight, based on said salts, of at least one of monomeric, dimeric and trimeric free higher fatty acids.

nitrogens, substantially all of which are in the form of amine salt groups with said alkylbenzene sulfonic acids, said amines selected from the group consisting of poly-

alkylene polyamines having 3-10 amino groups and 2-6 carbon alkylene groups and N-aminoalkyl substituted piperazines wherein the aminoalkyl group has the formula  $H(HNR—)_x$  wherein R is an alkylene group of 2-6 carbons and x is a small whole number, and (B) 10-150% by weight, based on said salts, of at least one of monomeric, dimeric and trimeric free higher fatty acids.

2. Compositions as claimed in claim 1 wherein said organic amines are polyalkylene polyamines having 3-10 amino groups and 2-6 carbon alkylene groups.

3. Compositions as claimed in claim 1 wherein said

free higher fatty acids consist essentially of dimer fatty acids.

4. Compositions as claimed in claim 1 wherein said free higher fatty acids consist essentially of dimer fatty acids and trimer fatty acids.

5. A method for inhibiting corrosion of ferrous metals in contact with corrosive media in corrosive oil compositions recovered from a subterranean formation which comprises treating said metals with oil containing corrosion inhibiting compositions comprising as the active, 45 corrosion inhibiting compounds (A) salts of (a) alkyl-

benzene sulfonic acids having 8-16 carbon alkyl groups and (b) partial amides of at least one of monomeric, dimeric and trimeric higher fatty acids and organic amines having a plurality of basic nitrogens, substantially all of which are in the form of amine salt groups with said alkylbenzene sulfonic acids, said amines selected from the group consisting of polyalkylene polyamines having 3-10 amino groups and 2-6 carbon alkylene groups and N-aminoalkyl substituted piperazines wherein the aminoalkyl group has the formula  $H(HNR—)_x$  wherein R is an alkylene group of 2-6 carbons and x is a small whole number, and (B) 10-150% by weight, based on said salts, of at least one of monomeric, dimeric and trimeric free higher fatty acids to provide corrosion inhibiting films on said metals.

6. A method as claimed in claim 5 wherein said free higher fatty acids consist essentially of dimer fatty acids.

7. A method as claimed in claim 5 wherein said free higher fatty acids consist essentially of dimer fatty acids and trimer fatty acids.

## References Cited

## UNITED STATES PATENTS

|           |        |                   |           |
|-----------|--------|-------------------|-----------|
| 2,290,154 | 7/1942 | Blair             | 252—344   |
| 2,598,213 | 5/1952 | Blair             | 252—392 X |
| 2,763,612 | 9/1956 | Raifsnider et al. | 252—8.55  |
| 2,791,495 | 5/1957 | Rudel et al.      | 252—389 X |

|           |         |                    |          |
|-----------|---------|--------------------|----------|
| 2,822,330 | 2/1958  | Riggs et al.       | 252—8.55 |
| 2,888,399 | 5/1959  | Wirtel et al.      | 252—8.55 |
| 2,941,943 | 6/1960  | Kirkpatrick et al. | 252—8.55 |
| 2,956,020 | 10/1960 | Suprin et al.      | 252—389  |
| 3,024,259 | 3/1962  | Sheldahl           | 252—8.55 |

HERBERT B. GUYNN, *Primary Examiner.*

UNITED STATES PATENT OFFICE  
CERTIFICATE OF CORRECTION

Patent No. 3,412,024

November 19, 1968

James R. Stanford

It is certified that error appears in the above identified patent and that said Letters Patent are hereby corrected as shown below:

Column 6, line 66, "40" should read -- 48 --.

Signed and sealed this 21st day of April 1970.

(SEAL)

Attest:

Edward M. Fletcher, Jr.

Attesting Officer

WILLIAM E. SCHUYLER, JR.

Commissioner of Patents